

## UNITED STATES PATENT OFFICE

2,265,138

DESENSITIZING OF LIGHT SENSITIVE  
SILVER HALIDE EMULSIONS

Emil Joachim Birr, Bitterfeld, Germany, assignor,  
by mesne assignments, to General Aniline &  
Film Corporation, New York, N. Y., a corpora-  
tion of Delaware

No Drawing. Application December 12, 1939, Se-  
rial No. 308,825. In Germany December 12,  
1938

12 Claims. (Cl. 95—88)

This invention relates to the desensitization of silver halide emulsions. It is a known fact to use anthraquinone derivatives for the desensitizing of photographic emulsions. Especially effective are taurides of the anthraquinonesulfo or carboxylic acids, especially anthraquinone acid amides, at least one hydrogen atom of the amide group being substituted by a radical, containing sulfo or carboxyl groups. According to the U. S. Patent No. 2,172,192, filed September 5, 1939, es-  
pecially ethers and thioethers of anthraquinone with aliphatic or aromatic radicals show excel-  
lent desensitizing qualities.

It has been found, that generally the qualities of the desensitizers of this class can be improved upon by using derivatives of anthraquinones, obtained by carbocyclic condensation with a triazole, as for instance anthraquinonetriazole, anthraquinonetriazolesulfo acid, anthraquinone-triazolecarboxylic acid, nitroanthraquinonetriazole etc., the two carbon atoms of the triazole nucleus condensed onto the anthraquinone nucleus being formed by two carbon atoms of one of the benzene rings of the anthraquinone nucleus. The sulfo acids of these new compounds of the typical formula



show a further increased effect compared with the substances hitherto known. At the same time these substances exhibit very favorable solubility and stability of the solutions and are not precipitated by calcium salts.

These compounds naturally may be added to the developer or may be used in preliminary baths.

*Example 1*

0.5 g. of 1,2-triazoleanthraquinone-3-sulfo acid are dissolved in one liter developer. In this developer ortho- or panchromatic photographic emulsions are developed one minute in the dark and thereafter finally developed in light green or yellow light.

*Example 2*

0.3 g. of 2,3-triazoleanthraquinone are dis-  
solved in one liter developer. The ortho- or  
panchromatic emulsions developed in this de-

veloper are, after a short development of 1-2 minutes in the dark, to be finally developed in light green or yellow dark-room light.

I claim:

- 5 1. A process for desensitizing light sensitive silver halide emulsions which comprises treating said silver halide emulsions with a compound formed by condensation of a triazole nucleus onto a carbocyclic ring of an anthraquinone nucleus.
- 10 2. A process for desensitizing light sensitive silver halide emulsions which comprises treating said silver halide emulsions with a compound formed by condensation of a triazole nucleus onto a carbocyclic ring of an anthraquinone nucleus selected from the group consisting of anthraquinone, anthraquinone sulfo acids, anthraquinone carboxylic acids and nitroanthraquinones.
- 15 3. A process for desensitizing light sensitive silver halide emulsions which comprises immersing said silver halide emulsions before development in an aqueous preliminary bath containing a compound formed by condensation of a triazole nucleus onto a carbocyclic ring of an anthraquinone nucleus.
- 20 4. A process for desensitizing light sensitive silver halide emulsions which comprises immersing said silver halide emulsions before development in an aqueous preliminary bath containing a compound formed by condensation of a triazole nucleus onto a carbocyclic ring of an anthraquinone nucleus selected from the group consisting of anthraquinone, anthraquinone sulfo acids, anthraquinone carboxylic acids and nitroanthraquinones.
- 25 5. A process for desensitizing light sensitive silver halide emulsions which comprises developing said silver halide emulsions in an aqueous solution of a developing agent and a compound formed by condensation of a triazole nucleus onto a carbocyclic ring of an anthraquinone nucleus.
- 30 6. A process for desensitizing light sensitive silver halide emulsions which comprises developing said silver halide emulsions in an aqueous solution of a developing agent and a compound formed by condensation of a triazole nucleus onto a carbocyclic ring of an anthraquinone nucleus selected from the group consisting of anthraquinone, anthraquinone sulfo acids, anthraquinone carboxylic acids and nitroanthraquinones.
- 35 7. As a desensitizer for light sensitive silver halide emulsions a compound formed by conden-

sation of a triazole nucleus onto a carbocyclic ring of an anthraquinone nucleus.

8. As a desensitizer for light sensitive silver halide emulsions a compound formed by condensation of a triazole nucleus onto a carbocyclic ring of an anthraquinone nucleus selected from the group consisting of anthraquinone, anthraquinone sulfo acids, anthraquinone carboxylic acids, nitroanthraquinones.

9. A bath for desensitizing light sensitive silver halide emulsions containing a compound formed by condensation of a triazole nucleus onto a carbocyclic ring of an anthraquinone nucleus.

10. A bath for desensitizing light sensitive silver halide emulsions containing a compound formed by condensation of a triazole nucleus onto a carbocyclic ring of an anthraquinone nucleus selected from the group consisting of anthraquinone, anthraquinone sulfo acids, anthra-

quinone carboxylic acids, and nitroanthraquinones.

11. A developer for developing light sensitive silver halide emulsion layers comprising an aqueous solution of a developing agent and a compound formed by condensation of a triazole nucleus onto a carbocyclic ring of an anthraquinone nucleus.

12. A developer for developing light sensitive silver halide emulsion layers comprising an aqueous solution of a developing agent and a compound formed by condensation of a triazole nucleus onto a carbocyclic ring of an anthraquinone nucleus selected from the group consisting of anthraquinone, anthraquinone sulfo acids, anthraquinone carboxylic acids and nitroanthraquinones.

EMIL JOACHIM BIRR.